

# United States Patent Office

2,736,709

Patented Feb. 28, 1956

1

2,736,709

## HYDRAULIC FLUIDS

Samuel A. Glickman and Joseph M. Wilkinson, Easton, Pa., assignors to General Aniline & Film Corporation, New York, N. Y., a corporation of Delaware

No Drawing. Application August 17, 1954,  
Serial No. 450,512

4 Claims. (Cl. 252—74)

This invention relates to hydraulic fluids and particularly to hydraulic brake fluids containing 3-methoxy-1-butanol and 3,5,x-polymethoxy-1-alkanols as the principal ingredients.

Many hydraulic fluid compositions are known to the art. The earliest improved fluids contained castor oil and a high boiling diluent in conjunction with various inhibitors. Later modifications included blown castor oil and castor oil glycol reaction products. However, low temperature usefulness, gum formation, and other factors led the art to find other materials.

When one surveys the field of organic liquids which could possibly be suitable for use as hydraulic fluids from the standpoint of viscosity at high and low temperatures, low volatility and lack of corrosive action on metals, etc., one is immediately impressed by the paucity of compounds which are acceptable from the standpoint of attack or the swelling of rubber. The vast majority of otherwise acceptable liquids including esters, ketones, halides, acetals, acids, amines, ethers, hydrocarbons, etc., have far too great a degree of rubber attack. As a result of many studies, it has been shown that very few organic liquids are acceptable in this respect. Outstanding among those acceptable are certain alcohols and ether alcohols having a favorable oxygen to carbon ratio and/or distribution in the molecule, i. e., structural configuration.

To be suitable for use as a hydraulic fluid, a liquid composition must have the following characteristics: It must not exhibit too great a viscosity change under wide temperature range, i. e., it must be reasonably viscous at the highest temperatures for which use it is contemplated, and on the other hand, it must remain fluid at the lowest temperatures likely to be encountered in automotive use, e. g., -50° F. In general, fluids which have a viscosity of at least 5 cps. at 130° F. and a viscosity no greater than 1500 cps. at -40° F. are considered suitable. A further requirement is that the fluid must have a lubricating action on most parts of the braking system in order to prevent undesirable wearing during use. In this respect, fluids which allow the moving parts to wear not more than .001 of an inch during 200,000 braking cycles are usually considered adequate.

It is an absolute prerequisite that a suitable fluid should not unduly attack any of the rubber or metal parts in the braking system. The attack on rubber is so undesirable that extensive research has gone into the manufacture of fluids which show a minimum of swelling or softening action on rubber. In regard to the attack on the metal parts, it might be said that the fluid must have the correct pH value, that is, presumably in the range of 8.5 to 9.5. In this range, protection would be obtained against the attack of acid sensitive metals, such as iron, tin, aluminum, zinc, etc. while this degree of alkalinity is not sufficiently high to cause the attack of alkali sensitive materials, such as aluminum and zinc.

It is a further prerequisite that the fluid should have as low a volatility as is practical to achieve, in order to eliminate the possibilities of evaporation from the brake

2

system storage unit as well as to prevent the undesirable evaporation of the fluid from the areas adjacent to hot braking surfaces. In the past, these objections have been achieved through the use of various mixtures of aliphatic alcohols, and glycerine esters, such as castor oil, soya oil, etc., or with mixtures of various ether alcohols, such as  $\beta$ -butoxy ethanol, the monoethyl ether of diethylene glycol and various polymers of ethylene oxide, propylene oxide, or interpolymers of ethylene and propylene oxides. The first-mentioned type consisting of alcohols and natural oils has certain shortcomings, e. g., with the lower aliphatic alcohols. The degree of attack on rubber rapidly increases with the increasing chain length of the alcohol used in practice. It has been found that alcohols higher than the butyl alcohols cannot be used because of excessive attack on, or swelling of, the rubber parts in the braking system. The alcohols up to and including the butyl alcohols have, unfortunately, rather low boiling points and hydraulic brake fluids prepared with them show an undesirably high degree of volatility. In addition, the presence of natural glycerine esters, such as castor oil and/or soya oil, etc., is undesirable because, as is well known, these substances are subject to oxidation and in time form undesirable gummy materials in the system. Because of the disadvantages, considerable effort has been made to develop improved fluids for hydraulic systems. One composition which has been suggested to overcome these disadvantages, comprises a mixture of the above-mentioned components: "Carbitol," butyl "Cellosolve," and interpolymers of ethylene oxide and propylene oxide.

While fluids of this type are better than mixture of alcohols and natural oils, they also have certain shortcomings. It has been established that the relatively low boiling points of two of the components used in such fluids, namely, butyl "Cellosolve" and "Carbitol," prevent such compositions from being considered for high temperature applications. It has been further established that such compositions will be prone to peroxide formation, a well known shortcoming characteristic of polyoxyethylenes, polyoxypropylenes, and the various interpolymers of ethylene oxide and propylene oxide.

We have found that the foregoing shortcomings and difficulties of the presently utilized fluids, particularly those containing polyoxyalkylenes and interpolymers of alkylene oxides are substantially overcome by employing an alkaline buffered mixture of 3-methoxy-1-butanol and 3,5,x-polymethoxy-1-alkanols as the principal ingredients with or without the presence of minor amounts of auxiliary components, such as anti-oxidants, corrosion inhibitors, viscosity regulators, and the like.

The 3-methoxy-1-butanol and 3,5,x-polymethoxy-1-alkanols utilized in the mixture are characterized by the following general formula:



where  $n$  represents an integer of from 1 to 10.

The alkanols characterized by the foregoing formula are prepared by reacting, in the known manner, vinyl methyl ether with methanol to yield dimethylacetal and reacting the latter with additional vinyl methyl ether. The ratio of methanol to vinyl methyl ether may vary from 2.0:1.0 to 20:1, preferably from 2.0:1 to 5.0:1, respectively. The crude acetal is then distilled to yield individual components which may be subjected to simultaneous hydrolysis-reduction to yield individual alkoxy-alkanols such as 3-methoxy-1-butanol; 3,5-dimethoxy-1-hexanol; 3,5,7-trimethoxy-1-octanol; 3,5,7,9-tetramethoxy-1-decanol; 3,5,7,9,11-pentamethoxy-1-dodecanol and polymethoxy-1-alkanols, as described in Examples 1, 4, and 5 of United States Patent 2,618,663. Alternatively,

the crude acetal may be subjected to simultaneous hydrolysis-reduction as described in Example 3 of said patent and the mixture of alkanols employed as such in accordance with the present invention. The mixture of alkanols may be distilled to yield the individual components of the alkanols and the individual components blended in the ratio of 20 to 40% of 3-methoxy-1-butanol and 60 to 80% of the remaining 3,5,x-polymethoxy-1-alkanols.

The alkanols are colorless liquids characterized by partial solubility in water, especially the methoxy derivatives which are completely soluble in water, and by complete miscibility in organic solvents, such as aliphatic alcohols, ketones, esters, glycol ethers, aromatic solvents, and aliphatic petroleum ethers and naphthas. The complete miscibility in aliphatic hydrocarbons is in sharp distinction to the polyethylene glycols which are virtually insoluble in these solvents.

All of the alkanols in the mixture, i. e., the 3-methoxy-1-alkanol and 3,5,x-polymethoxy-1-alkanols, when in contact with rubber have a very low swelling action, considerably less than that tolerated by commercially available hydraulic fluids. In addition they possess an unusual inertness to oxidation attack. It is believed that the arrangement of atoms in the alkanols of the mixture contributes to this property. This is unexpected since it has been recognized by the art, U. S. P. 2,492,955 and 2,481,278, that polymers of ethylene and propylene oxide have one serious drawback which limits their use as lubricants because the two carbon unit between the ether linkage in the polymer chain appears to make the polymer extremely sensitive to oxidation.

The hydraulic fluids prepared in accordance with the present invention possess sufficient lubricity under operating conditions in various climes and extremes of temperatures. Tests have indicated that the lubricity is met by the presence, even in very small amounts, of the higher members of the 3,5,x-polymethoxy-1-alkanols series which are viscous liquids resembling glycerine and the low polyethylene glycols in consistency. These materials are free from gum formation which is a serious drawback to the use of lubricants of the like of castor oil and derived compounds.

The presence in the hydraulic fluid of low boiling diluents either as solvents or decomposition products may result in vapor lock and is, therefore, to be avoided. The lowest member of the alcohol series is 3-methoxy-butanol with a boiling point of 159° C. at 760 mm. The presence of the higher members of the series increases the pot temperature at which such a mixture boils and may be varied depending on needs.

The wide solvent power of the 3,5,x-polymethoxy-1-alkanols makes it possible to secure homogeneous solutions on mixing with commercial hydraulic fluids. The water tolerance of the 3,5,x-polymethoxy alkanols is excellent.

The hygroscopicity of the 3,5,x-polymethoxy-1-alkanols is of a lower order than the glycols and polyethylene glycols in the same molecular weight range. Brake fluid mixtures containing these alkanols possess advantages over materials containing the polyethylene glycols.

Inasmuch as mixtures of 3-methoxy-1-alkanols and 3,5,x-polymethoxy-1-alkanols may in themselves serve as hydraulic brake fluids because of their desirable properties, it is at times desirable to fit certain needs to incorporate auxiliary substances, such as anti-oxidants, corrosion inhibitors, viscosity modifiers, buffering agents, and the like.

As anti-oxidants, there may be used any of the materials commonly used to prevent the oxidation of oxidizable organic compounds, such as unsaturated hydrocarbons, e. g., rubber, unsaturated fuels, unsaturated esters, such as oxidizable vegetable oil, ethers, vinyl compounds, etc. Examples of these anti-oxidants are para-tertiary butyl-

catechols, hydroquinones, and various morpholine derivatives, such as N-phenyl-morpholine, N-(p-hydroxyphenyl)morpholine, N,N - diphenyl-p-phenylenediamine, diphenylamine, N - phenyl- $\beta$ -naphthylamine, p-phenylphenol, o-phenylphenol, di-p-methoxydiphenylamine, m-toluylenediamine, various condensation products of aldehydes with aromatic amines: acetone-aniline and acet-aldehyde - aniline and butylaldehyde-aniline, aldol- $\beta$ -naphthylamine, hydroquinone monobenzyl ether, and isopropoxydiphenylamine.

As corrosion inhibitors, we may use inorganic nitrites, such as sodium nitrites, etc., organic nitrites, such as tertiary amine nitrites, chromates, such as sodium chromates and the like, inorganic boron compounds, such as sodium tetraborate, organic boron compounds, such as triethanol amine borate and the like, certain sulfur compounds, such as dialkylthiourea, mercaptans, organic disulfides, diarylamine phosphates, such as diphenylamine phosphate, long chain alkyl sulfonamide acetate sodium salt, phosphites, such as sodium phosphite, organic phosphoric acid and organic derivatives of phosphorous acids, such as benzene-phosphoric acid, etc.

In addition to the components named above, auxiliary substances, such as viscosity modifiers, buffering agents, and coloring agents may be optionally added.

As viscosity modifiers, there may be used various polyhydroxy compounds, such as glycol, glycerine, 1,2,4-butanetriol, 1,4-butanediol, propylene glycol, etc., especially when used in conjunction with complex forming inorganic salts, such as borax, nickel and chromium salts, various polymeric materials, such as polyvinyl methyl ether, polyvinyl butyl ether, interpolymers of isobutyl vinyl ether and oleyl vinyl ether, various polyacrylates, such as polylauryl acrylate, polyolefines, such as polyisobutylene or interpolymers thereof, etc.

As buffering agents, the following inorganic compounds are useful: borates, such as sodium tetraborate, sodium metaborate, ammonium and organic borates, such as triethanolamine borates, sodium phosphite, tetraborate and the like, inorganic phosphate, such as the various sodium phosphates, such as trisodium o-phosphate, disodium hydrogen phosphate, sodium pyrophosphate, organic phosphate, e. g., triethanolamine phosphate, quinoline phosphate, salts of alkaline metals, organic acids, such as sodium acetate, sodium citrate, sodium benzoate, potassium tartrate and the like, and mixtures thereof to yield (when admixed in the brake fluid composition) a pH above 7 and not exceeding a pH of 11.

In order to dissolve sodium borate in the hydraulic brake fluid composition, it was found advantageous to use a solubilizing agent, such as ethylene glycol, in the formation. However, glycol is not essential in the hydraulic brake fluid. This agent can be omitted in compositions in which other buffers are incorporated. Also in place of ethylene glycol in borax formations, other solubilizing agents, such as "Carbitol" can be used.

The choice of coloring matter is not of critical importance in the finishing of the hydraulic brake fluid provided it does not cause a deleterious effect on the viscosity of the fluid or exhibit corrosive action on the rubber or metal parts of the braking system. Most dyestuffs are acceptable on these accounts since in most cases they are used only in minute quantities. Where coloring material or dyestuffs are added for identification or other purposes, the sole requirement is that the dyestuff be sufficiently soluble in the hydraulic fluid. It has been found that dyestuffs of any class may be used. These include vat dyestuffs, diphenylamine derivatives, azo dyes, triphenylmethane dyes, and the like.

From the standpoint of rubber swelling, we have found that the proportions of 3-methoxy-1-butanol in the mixture must range from 20 to 40% to yield good results. The 3-methoxy-1-butanol does not appear to give good results when employed alone or when incorporated with the foregoing auxiliary substances. The unusual and

## 5

unexpected feature of the present invention is that the mixture, in addition to 20-40% of 3-methoxy-1-butanol, must contain 60 to 80% of at least one of the individual 3,5,x-polymethoxy-1-alkanols or a mixture thereof to yield good results. In these proportions the brake fluid does not cause any swelling or disintegration of rubber and completely eliminates brake failure through loss of fluid. Moreover, the blending of the individual alkanols of the mixture makes it readily possible to fit prescribed commercial needs or requirements of certain brake fluids with respect to non-volatility, viscosity, lubricity, and miscibility with auxiliary components. For general all around good results particularly in automotive hydraulic brake fluids, we have found that the following blend is ideal:

|                                     | Percent |
|-------------------------------------|---------|
| 3-methoxy-1-butanol                 | 20-40   |
| 3,5-dimethoxy-1-hexanol             | 25-35   |
| 3,5,7-trimethoxy-1-octanol          | 15-30   |
| 3,5,7,9-tetramethoxy-1-decanol      | 5-20    |
| 3,5,7,9,11-pentamethoxy-1-dodecanol | 2.5-10  |
| 3,5,7,9,11,13- and higher           | 0.5-3.5 |

The following blend may also be used for all around good results:

|                                     | Percent |
|-------------------------------------|---------|
| 3-methoxy-1-butanol                 | 20-35   |
| 3,5-dimethoxy-1-hexanol             | 25-35   |
| 3,5,7-trimethoxy-1-octanol          | 10-25   |
| 3,5,7,9-tetramethoxy-1-decanol      | 5-20    |
| 3,5,7,9,11-pentamethoxy-1-dodecanol | 2.5-10  |

Polymethoxy-1-alkanols characterized by the following formula:



wherein  $n$  represents an integer of from 6 to 8, 0.5-3.5%.

The higher polymethoxy alcohols of the type 3,5,7,9-, 11,13,x-polymethoxy-1-alkanols, i. e., wherein  $n$  in the above formula equals 6 or greater, may be used in the range of 60 to 80% to 20 to 40% of 3-methoxy-1-butanol to yield a mixture which gives excellent results with respect to prevention of rubber swelling. A mixture of 20% of 3-methoxy-1-butanol and 80% of 3,5-dimethoxy-1-hexanol is comparable to a mixture of 40% of 3-methoxy-1-butanol and 60% of 3,5-dimethoxy-1-hexanol. Both mixtures possess sufficient lubricity under operating conditions in various climates and extremes of temperatures.

As illustrative of the preparation of hydraulic brake fluids in accordance with the present invention, the following examples are given. The parts are by weight.

## EXAMPLE I

To 88.6 parts of a mixture of 3,5,x-polymethoxy alkanol (prepared in accordance with Example 3, United States Patent 2,618,663), containing by weight the following components:

|                                                                                   | Percent |
|-----------------------------------------------------------------------------------|---------|
| 3-methoxy-1-butanol                                                               | 35.0    |
| 3,5-dimethoxy-1-hexanol                                                           | 30.0    |
| 3,5,7-trimethoxy-1-octanol                                                        | 22.0    |
| 3,5,7,9-tetramethoxy-1-decanol                                                    | 7.5     |
| 3,5,7,9,11-pentamethoxy-1-dodecanol                                               | 3.6     |
| Higher homologues characterized by the above formula wherein $n$ equals 6 or more | 2.9     |

A solution of 1 part of borax, 0.3 part of N-phenylmorpholine, and 0.1 part of an organic nitrite corrosion inhibitor (sold under the trade name "V. P. I. 260 Crystals") in 10 parts of ethylene glycol was added. The resulting mixture was stirred until it became a homogeneous solution.

The viscosity of the composition at -40° F. was 1150 cps. and at +130° F. was 7 cps. A tube containing this material was maintained at -40° F. for 6 days and at

## 6

the end of this period, the tube was tilted from a vertical to a horizontal position. It was observed that flow began immediately. This composition was maintained at -60° F. for 6 hours. Flow began immediately upon tilting. The material was admixed 10% by weight with water and maintained at -60° F. for 6 hours after which it was clear and fluid. The boiling point as determined by the temperature of the reflux was found to be 345° F. Flash point by Cleveland open cup ASTM method was 180° F. A sample of the fluid was weighed into a ceramic boat and maintained at 210° F. for 48 hours in a location free from drafts. Only 70% of the fluid evaporated. The pH was determined using a Beckman pH meter and found to be 9.3. A sample was boiled under a reflux condenser at its atmospheric boiling point of about 345° F. for 8 hours. At the conclusion of this treatment the material showed only a very slight yellowing. No other evidence of decomposition was noted, and the sample was judged to be remarkably stable. This composition was admixed with other commercially available brake fluids, for example, a fluid composed of about 35% by volume of ethylene oxide-propylene oxide interpolymers, 32.5% by volume of butyl "Cellosolve" and 32.5% by volume of "Carbitol" in addition to various inhibitors and found to be completely miscible within the temperature range of -30 to +60° F.

A 1 1/4 inch Wagner-Lockheed FC666 wheel cylinder cup was measured to the nearest thousandth inch and introduced into this composition at a temperature of 158° F. for a period of 120 hours. Afterwards, the cup was again measured and the increase in diameter due to the swelling effects of the composition was 0.018 inch. The above composition was brought in contact with all the parts of a commercial wheel brake cylinder and maintained at 158° F. for 14 days. Upon disassembly and examination, it was found that the fluid caused no rust or corrosion of the metal parts and left no hard, dry gummy residue or any substantial amount of sludge. Test strips of tinned iron, cold rolled steel, aluminum, cast iron, brass and copper were bolted together so that the strips were in electrical contact. These strips and a part of a sample taken from a Wagner-Lockheed FC666 rubber wheel cylinder cup were introduced into the above composition, diluted with 5% by volume of distilled water, maintained at a temperature of 210° F. for 120 hours. At the end of this period the strips were removed, disengaged and polished to remove corrosion products, if any. Corrosion losses were observed by noting the weight lost (milligram per square cm.):

|          | Loss                      |
|----------|---------------------------|
| Tin      | 0                         |
| Steel    | 0                         |
| Brass    | 0                         |
| Copper   | milligram per sq. cm. 0.1 |
| Aluminum | 0                         |
| Iron     | milligram per sq. cm. 0.1 |

A lubrication test was carried out in a commercial hydraulic brake wheel cylinder actuated by a conventional mast cylinder driven by a cam. The assembly was operated to simulate the actual actions of a brake in normal operation and the wheel cylinder was actuated in this fashion every six seconds. The composition of Example I was introduced into this system and underwent 160,000 braking cycles at the completion of which the moving parts were disassembled and examined for evidence of wear. Wearing was determined visually and by micrometer measurements. None of the surfaces exhibited as much as 0.001 inch wear.

## EXAMPLE II

To the same solution of the composition of Example I there were added 20 parts per million of a soluble copper phthalocyanine dyestuff. The performance data for this colored composition was substantially identical with that

as above indicating that the colorant had no deleterious effect. The presence of colorant is often desirable to aid in the detection of leaks in a hydraulic system.

## EXAMPLE III

To 99.5 parts of the mixed polymethoxyalkanol of the composition of Example I, there were added 0.4 part of copper naphthenate and 0.1 part of triethanolamine. The mixture was stirred until a homogeneous solution resulted. This composition exhibited a viscosity of 420 cps. at a temperature of  $-40^{\circ}$  C. and a viscosity of 16 cps. at  $+25^{\circ}$  C. When a Wagner-Lockheed FC666 wheel cylinder rubber cup was immersed in this composition for a period of 24 hours at  $158^{\circ}$  F., the cup showed, after an alcohol rinse and drying, a weight increase of only 8.8%.

By way of comparison,  $\beta$ -butoxyethanol often used as a constituent in commercial brake fluid exhibited a rubber swell of 37.4%.

## EXAMPLE IV

A brake fluid composition was prepared by dissolving one-tenth part of triethanolamine, 0.3 part of p-hydroxy-phenylmorpholine and 0.1 part of the amine nitrite described in Example I, in 99.5 parts of a mixture of polymethoxyalkanols of Example I. The compounding was carried out by stirring the constituents together at room temperature until a homogeneous mixture resulted. When test strips of cast iron, steel, tin, iron, brass, copper and aluminum were immersed in the composition for a period of 5 days at  $100^{\circ}$  C., it was found in all cases that the weight loss of the strips due to corrosion was less than 0.3 milligram per square centimeter. An average corrosion value of 0.5 mg. per sq. cm. over the above described test condition for these metals is normally considered excellent.

## EXAMPLE V

A solution of 0.5 part of borax, 0.3 part of phenyl- $\beta$ -naphthylamine, and .01 part of sodium nitrite in 25 parts of ethylene glycol was added with stirring to 75 parts of the mixed polymethoxyalkanols of Example I. The resulting mixture was agitated until homogeneous. In a rubber swelling test in which a 1 $\frac{1}{4}$  inch Wagner-Lockheed FC666 wheel cylinder rubber cup was immersed in this composition for 120 hours at  $70^{\circ}$  C., the diameter of increase of the rubber cup was 0.018 inch. In a commercially marketed fluid consisting of essentially 65% n-butanol and 35% castor oil together with suitable stabilizers, the rubber swell in the same test was found to be 0.22 inch.

## EXAMPLE VI

Four samples of crude polymethoxyacetals, obtained by reacting vinyl methyl ether with various ratios of methanol, were subjected to simultaneous hydrolysis-reduction in accordance with the steps of Example 3 of U. S. P. 2,618,663 to yield a concentrate (mixture of alkanols). The concentrate of each sample was divided in two. The first four separate samples were set aside and the second four subjected to distillation. The percentage by weight of the individual alcohols obtained from the second four samples is shown in the following table:

Polymethoxy alkanols obtained from polymethoxyacetals

| Vinyl Ether to Methanol Ratio of Polymethoxyacetal | 2.6:1   | 2.8:1   | 2.9:1   | 3.0:1   |
|----------------------------------------------------|---------|---------|---------|---------|
| Component:                                         | Percent | Percent | Percent | Percent |
| 3-methoxy-1-butanol                                | 34.3    | 27.8    | 23.2    | 23.8    |
| 3,5-dimethoxy-1-hexanol                            | 29.7    | 28.9    | 31.2    | 27.5    |
| 3,5,7-trimethoxy-1-octanol                         | 22.2    | 24.8    | 26.4    | 21.3    |
| 3,5,7,9-tetramethoxy-1-decanol                     | 7.5     | 12.9    | 12.1    | 18.3    |
| 3,5,7,9,11-penta-1-methoxydodecanol                | 3.6     | 4.3     | 4.5     | 8.0     |
| 3,5,7,9,11,13- and higher                          | 2.6     | 3.0     | 3.0     | 3.2     |

65

70

75

## EXAMPLE VII

To each of the first set of four samples (which were set aside) each weighing about 90 parts, there was added a solution of 0.6 part of borax, 0.35 part of phenyl- $\beta$ -naphthylamine, and 0.03 part of sodium nitrite in 30 parts of ethylene glycol. The resulting four mixtures were agitated until homogeneous. In rubber swelling tests in which a 1 $\frac{1}{4}$  inch Wagner-Lockheed FC666 wheel cylinder rubber cup was immersed in each of the four compositions for 120 hours at  $70^{\circ}$  C., the diameter of increase of the rubber cup was 0.012".

## EXAMPLE VIII

Example IV was repeated with the exception that 99.5 parts of the mixture of polymethoxyalkanols of Example I were replaced by 95 parts of a mixture consisting of 40% of 3,5-dimethoxy-1-hexanol and 60% of 3,5,7,9,11-pentamethoxy-1-dodecanol prepared in accordance with Examples 1 and 4 respectively, of U. S. P. 2,618,663. When the compounded mixture was subjected to the corrosion strip test, the weight of loss of the strips due to corrosion was less than 3.3 milligrams per cm.

## EXAMPLE IX

Example III was repeated with the exception that 99.5 parts of methoxyalkanols of the composition of Example I were replaced by 75 parts of a mixture consisting of 20% of 3-methoxy-1-butanol and 80% of 3,5,7-trimethoxy-1-octanol prepared in accordance with Examples 1 and 5 respectively, of U. S. P. 2,618,663. When a Wagner-Lockheed FC666 wheel cylinder rubber cup was immersed in this composition for a period of 120 hours at  $133^{\circ}$  C., the cup showed, after an alcohol rinse and drying, a weight increase of only 8.3%.

This application is a continuation-in-part of our application Serial No. 227,540, filed on May 21, 1951, now abandoned.

We claim:

1. A hydraulic fluid composition consisting essentially of an alkaline buffering agent selected from the class consisting of alkaline borates, phosphates and phosphites, and a mixture of mono- and polymethoxy-1-alkanols consisting of 20 to 40% of 3-methoxy-1-butanol and 60 to 80% of at least one 1-polymethoxy-alkanol of the group consisting of 3,5-dimethoxy-1-hexanol, 3,5,7-trimethoxy-1-octanol, 3,5,7,9-tetramethoxy-1-decanol, 3,5,7,9,11-pentamethoxy-1-dodecanol, and polymethoxy-1-alkanols characterized by the following formula:



wherein  $n$  represents an integer of from 6 to 10.

2. A hydraulic fluid composition consisting essentially of an alkaline buffering agent selected from the class consisting of alkaline borates, phosphites, and phosphates, and a mixture of mono- and polymethoxy-1-alkanols consisting of 20 to 35% of 3-methoxy-1-butanol, 25 to 35% of 3,5-dimethoxy-1-hexanol, 10 to 25% of 3,5,7-trimethoxy-1-octanol, 5 to 20% of 3,5,7,9-tetramethoxy-1-decanol, 2.5 to 10% of 3,5,7,9,11-pentamethoxy-1-dodecanol, and 0.5 to 3.5% of polymethoxy-1-alkanols characterized by the following formula:



wherein  $n$  represents an integer of from 6 to 8.

3. A brake fluid composition consisting essentially of an alkaline buffering agent selected from the class consisting of alkaline borates, phosphites, and phosphates, and a mixture of mono- and polymethoxy-1-alkanols consisting of 35.0% of 3-methoxy-1-butanol, 30.0% of 3,5-dimethoxy hexanol, 22.0% of 3,5,7-trimethoxy-1-octanol, 7.5% of 3,5,7,9-tetramethoxy-1-decanol, 3.6% of

**9**

3,5,7,9,11-pentamethoxy-1-dodecanol, and 2.9% of polymethoxy-1-alkanols having the following formula:



5

wherein  $n$  represents an integer of from 6 to 8.

4. A brake fluid composition consisting essentially of an alkaline buffering agent selected from the class consisting of alkaline borates, phosphites, and phosphates, and a mixture of mono- and polymethoxy-1-alkanols consisting of 10 to 20 to 40% of 3-methoxy-1-butanol, 25 to 35% of 3,5-dimethoxy-1-hexanol, 15 to 30% of 3,5,7-trimethoxy-1-octanol, 5 to 20% of 3,5,7,9-tetramethoxy-1-decanol, 2.5 to 10% of 3,5,7,9,11-pentamethoxy-1-dodecanol, and 0.5

**10**

to 3.5% of polymethoxy-1-alkanols characterized by the following formula:



wherein  $n$  represents an integer of from 6 to 10.

## References Cited in the file of this patent

## UNITED STATES PATENTS

|    |           |                 |               |
|----|-----------|-----------------|---------------|
| 10 | 2,165,962 | Mueller-Cunradi | July 11, 1939 |
|    | 2,481,278 | Ballard et al.  | Sept. 6, 1949 |
|    | 2,564,760 | Hoaglin et al.  | Aug. 21, 1951 |
|    | 2,564,761 | Hoaglin et al.  | Aug. 21, 1951 |
|    | 2,618,663 | Glickman et al. | Nov. 18, 1952 |